

Patented Apr. 8, 1924.

1,489,356

# UNITED STATES PATENT OFFICE.

WILLIAM J. McELROY, OF NEW YORK, AND JOHN CLARKE, OF MANHASSET, NEW YORK,  
ASSIGNORS, BY MESNE ASSIGNMENTS, TO ALCHEMIC GOLD COMPANY, INC., A COR-  
PORATION OF NEW YORK.

## PRINTING INK.

No Drawing.

Application filed May 20, 1922. Serial No. 562,437.

*To all whom it may concern:*

Be it known that we, WILLIAM J. McELROY, a citizen of the United States, and a resident of the borough of Manhattan, city, <sup>5</sup> county, and State of New York, and JOHN CLARKE, a citizen of the United States, and a resident of the village of Manhasset, town of North Hempstead, county of Nassau, and State of New York, have invented a new <sup>10</sup> and useful Improvement in Printing Inks, of which the following is a description, as well as of the manner and process of making, constructing, compounding, and using the same, in such full, clear, concise, and <sup>15</sup> exact terms as to enable any person skilled in the art or science to which it appertains or with which it is most nearly connected to make, construct, compound, and use the same.

<sup>20</sup> Our invention relates generally to printing inks and particularly to those having metallic powders as their pigments.

The objects of our invention are the production of improved printing inks adapted <sup>25</sup> for general use and more especially for use in embossing and die-printing upon book-cloth, leather and other materials commonly used for book-casings; particular objects are the production of inks of this class which <sup>30</sup> shall be adapted for application by a heated die, plate or other impression member, preheated to embossing temperatures, and which shall be characterized by the qualities of drying immediately under the relatively <sup>35</sup> high temperature preferred in embossing metallic powders; and having properties of strongly adhering to and covering smoothly, evenly and completely the surface upon which they are stamped; of being rendered <sup>40</sup> lustrous by the heat of the metal by which they are impressed upon such object; of permanently retaining their original color and luster without tarnishing or fading; of high boiling point and of low volatility.

<sup>45</sup> Further objects are the provision of an ink with the foregoing qualities which can be mixed ready for use by the manufacturer and which will not corrode or otherwise deteriorate in the container, and which, <sup>50</sup> when packaged, and transported shall remain in its original state with its qualities and both its physical and chemical conditions unimpaired even after long lapse of time.

Heretofore it has been proposed to make <sup>55</sup> an ink having metallic pigments such as bronze powders incorporated therein, employing a vegetable wax as a binder for the metallic powders and a solvent for the binder, but it has been found that the acidic <sup>60</sup> solvents employed caused the bronze powders to corrode; also that the acid solvent vehicle evaporated quickly, leaving the residue a hardened mass difficult to reclaim; and further, that the characters and patterns embossed or otherwise printed therewith rubbed or even flaked off.

It has also been proposed to employ a resin as a binder in lieu of wax, with a suitable solvent therefor. It has been found, <sup>70</sup> however, that due to the acid content of the resins, the metallic powders soon became corroded. These ingredients cannot, therefore, be combined by the manufacturer and sold as a ready-mixed ink. It is necessary to package the metallic pigment separately from the binder and its vehicle solvent and to delay mixing them to form the ink desired until the printer is ready to use it. This devolves upon the user a mixing <sup>75</sup> operation which, by reason of the fine state of division of the metallic pigment, requires time, labor and skill to produce a homogeneous, correctly proportioned ink of the right consistency.

Our invention attains the above recited features of advantage while avoiding the disadvantages inherent in inks of the acid-constituent class described.

With the foregoing desired objects in view <sup>90</sup> and others hereinafter developed, our invention, broadly stated, consists in the discovery of a printing ink composed of metallic powders and a neutral binder dissolved in a neutral solvent, which solvent has <sup>95</sup> a high boiling point and low volatility.

All resins are acid. Otherwise most of the resins possess qualities desirable in a binder, particularly the capacity to coat or encase the comminuted particles composing the metallic pigments when printed and thereby protect the printed ink from discoloration by contact with atmospheric gases. Of the resins, white rosin is especially suitable except for the abietic acid constituting its normal major constituent, which renders it a bronze powder corrosive. By esterification of the rosin with a glyceryl

radical, the abietic acid is neutralized. This product is known commercially as "ester gum". It is soluble in resin solvents, though not itself a resin, and readily soluble in terpineol, which is also non-acid. Other resins and rosins may be similarly treated to obtain their esters.

Most resin solvents have a boiling point so low that they cannot be used with a die 10 heated to the temperature requisite to impart to the metallic pigments the desired lustrous appearance of burnished metal when stamped or embossed. Many of them are acid. Most of them have color. Terpineol is neutral as to acidity; is colorless; and has a sufficiently high boiling point to work satisfactorily at the temperatures desired to cause the metallic deposit to adhere firmly to the book-cover by fluxing the resin 15 ester, and by such fluxing to coat the metallic deposit with a protective film thereof, rendering it gas and waterproof, and to impart a maximum luster to the pigment. The comparatively low volatility of terpineol renders it advantageous as a vehicle for the mixture of metallic powders and dissolved binder because the mixed ink retains its desired consistency, and will not cake or harden upon exposure. As an example of the preferred proportions of the ingredients named:

Dissolve from 10 to 20 per cent by weight of ester gum in from 80 to 90 per cent by weight of terpineol. Take two parts of 35 bronze powder to one part of the gum solution, also by weight, and mix thoroughly.

The commercial purity of the ingredients varies somewhat. With the particular grades of ingredients to be named, the proportions preferred are as follows:

With L. Hemmerdinger & Co.'s "Special No. 1" bronze powder, use Eimer & Amend's terpineol, 84 per cent, and Charles F. Gledhill's "ester gum", 16 per cent.

45 The compound, when mixed, is ready for use as an ink. It is of the usual consistency of printing inks, a pasty semi-liquid. It does not clog the types or dies and dries immediately under the heat of the impression head.

We have further found that the covering 50 properties of the bronze powders are improved if re-enforced with a superlative grade thereof known commercially as "lining". "Lining" is a bronze powder reduced to a finer stage of subdivision. For example, to 80 per cent of the "Special No. 1" bronze powder, above specified, we add 20 per cent of "lining", by weight, the binder

and vehicle remaining unchanged in proportionality.

The above mixture is adapted for use at the preferred embossing temperature afforded by the "high" of the electric heater attachment supplied with their standard 60 presses of the "Universal" type by the John Thomson Press & Manufacturing Company, approximately 500° Fahr., or with the presses of the Markem Machine Company, as described in their patent to Putnam, No. 70 1,108,518, of August 25, 1914, for machine for embossing or marking leather.

It will be obvious to those skilled in the art that the term "bronze-powders" as herein employed comprehends all the metallic 75 powders used as pigments.

While we prefer the particular features of utility and advantage attained by working the described ink with a heated impression head, we do not intend to be understood 80 as limiting our novel ink thereto, since it is adapted for use as are the ordinary inks used in printing, and works well when used cold upon paper and the like.

Having thus described the preferred embodiment of our invention and the best method now known to us of producing the same, we claim:

1. A printing ink suitable for application with a heated die, composed of a resin ester, a neutral solvent and a metallic pigment.

2. A printing ink suitable for application with a heated die, composed of an ester of rosin, a neutral solvent and a metallic pigment.

3. A printing ink composed of an ester of white rosin, a neutral solvent and a metallic pigment.

4. A printing ink composed of a resin ester, terpineol and a metallic pigment.

5. A printing ink composed of an ester of rosin, terpineol and a metallic pigment.

6. A printing ink composed of an ester of white rosin, terpineol and a metallic pigment.

7. A printing ink consisting of two parts of metallic pigment and one part of a binder solution containing between 10 and 20 per cent of a neutralized resin and between 80 and 90 per cent of a neutral solvent therefor, both by weight.

8. A printing ink consisting of two parts of bronze powder and one part of a binder solution containing 16 per cent of ester gum and 84 per cent of terpineol, both by weight.

WILLIAM J. McELROY.  
JOHN CLARKE.